

3,600,313

COBALT CHROMIUM SULFIDE MAGNETIC COMPOSITIONS HAVING A PYRITE TYPE STRUCTURE AND DEVICES CONTAINING SAME  
Paul Christopher Donohue, Wilmington, Del., assignor to E. I. du Pont de Nemours and Company, Wilmington, Del.  
No Drawing. Filed Oct. 31, 1969, Ser. No. 873,064  
Int. Cl. C04b 35/00; H01v 3/00; H01b 37/32  
U.S. Cl. 252—62.51

6 Claims

## ABSTRACT OF THE DISCLOSURE

Magnetic pyrite-type phases having the formula



where  $x=0.01$  to  $0.4$ . The compositions are useful in magnetic switching devices, temperature sensing devices, and the like.

## BACKGROUND OF THE INVENTION

### Field of the invention

This invention relates to magnetic pyrite-type phases having the formula  $\text{Co}_{1-x}\text{Cr}_x\text{S}_2$  where  $x$  is  $0.01$  to  $0.4$ .

### Description of prior art

Chromium forms a series of sulfides from  $\text{CrS}$  to  $\text{Cr}_{1.6}\text{S}_2$  which have crystalline structures related to those known in the art as the nickel-arsenide type.  $\text{Cr}_{5}\text{S}_6$  is ferromagnetic with a Curie temperature ( $T_c$ ) of  $303^\circ\text{K}$ . There is no compound of the formula  $\text{CrS}_2$ .

The only compound known in the  $\text{Co/Cr/S}$  system is  $\text{CoCr}_2\text{S}_4$ . It has spinel-type structure and is ferromagnetic with  $T_c$  of  $240^\circ\text{C}$ .

$\text{CoS}_2$  has been reported to have the pyrite-type structure and to exhibit metallic-type electrical conduction. It is ferromagnetic with a  $T_c$  of  $118^\circ\text{K}$ . and saturation magnetization ( $\sigma_s$ ) of about 41.5 electromagnetic units (emu.) per gram. No substitution of Cr in  $\text{CoS}_2$  has been reported. However, when other transition metal sulfides, specifically  $\text{FeS}_2$  and  $\text{NiS}_2$ , have been combined at ambient pressure with  $\text{CoS}_2$  to form solid solutions, the Curie temperature and saturation magnetization generally decrease to zero as the amount of iron or nickel is increased. (Both  $T_c$  and  $\sigma_s$  increase slightly with initial iron substitution into  $\text{CoS}_2$  before decreasing to zero with further additions of Fe. Maxima for these two parameters occur at  $T_c \approx 146^\circ\text{K}$ . for  $\text{Co}_{0.75}\text{Fe}_{0.25}\text{S}_2$  and  $\sigma_s \approx 43$  emu./g. for  $\text{Co}_{0.95}\text{Fe}_{0.05}\text{S}_2$ .)

## DESCRIPTION OF THE INVENTION

The compositions of this invention have the formula  $\text{Co}_{1-x}\text{Cr}_x\text{S}_2$  where  $x$  is  $0.01$  to  $0.4$ . They have the pyrite-type structure and are magnetic with the magnitude of  $T_c$  increasing with the Cr content and the magnitude of  $\sigma_s$  decreasing with it. For example, when  $x=0.05$ ,  $T_c=177^\circ\text{K}$ . and  $\sigma_s=36.53$  emu./g. while when  $x=0.25$ ,  $T_c=343^\circ\text{K}$ . and  $\sigma_s=16.32$  emu./g. The cubic cell dimension,  $a$  increases with increasing Cr content.

The phases are prepared by reaction of the elements or sulfides of Cr and Co mixed to produce the desired composition of the phase. To enhance reaction and impede the formation of  $\text{Cr}_2\text{S}_3$ , excess S is useful in the reaction mixture.

The reagents should be thoroughly mixed. Reactions are carried out at  $650^\circ\text{C}$ . to  $1300^\circ\text{C}$ . and 1 atmosphere to 65 kilobars (kb.). Preferred conditions are  $1100^\circ\text{C}$ .  $1200^\circ\text{C}$ . and 30 to 65 kb.

For high pressures and temperatures, a tetrahedral anvil pressure device as described by E. C. Lloyd et al., J. of Research, National Bureau of Standards, 63C, 59

(1959) can be used. In the device the prepelleted reactants are placed in a boron nitride container which is fitted into a graphite sleeve that serves as a resistance heater. This assembly is enclosed in a pyrophyllite tetrahedron and placed in the anvil device capable of generating pressures in excess of 65 kb.

Four of the calibration points taken at room temperature used to determine pressure developed in this device appear in the 1963 edition of the American Institute of Physics Handbook, pp. 4-43 as follows:

Bismuth I $\rightarrow$ II  $25.37 \pm 0.02$  kb.

Bismuth II $\rightarrow$ III  $26.96 \pm 0.18$  kb.

Thallium II $\rightarrow$ III  $36.69 \pm 0.11$  kb.

Barium II $\rightarrow$ III  $59.0 \pm 1.1$  kb.

15 All compressions are made on the cold assembly and the charges then heated to the desired temperature, measured with an appropriate thermocouple. No pressure correction for thermocouple behavior has been introduced; standard electromagnetic force (EMF) tables for one atmosphere were used. The temperatures are measured at the center of the external surface of the boron nitride crucible. The temperature at the ends is approximately  $30^\circ$  cooler.

20 The reaction conditions employed generally involve a slow cool to enhance crystal growth. The crystals generally grow at the ends of the pellet in the form of black rods. In such cases separation from excess S or excess  $\text{Cr}_2\text{S}_3$  was done mechanically. Samples were washed with carbon disulfide to remove further excess sulfur.

25 The products of all reactions were examined by Debye-Scherrer X-ray powder techniques. The cubic unit cell dimension of the pyrite-type phase was refined using a computerized least squares technique in which the Nelson-Riley function is one of the parameters. When single-phase

30 material was separable from a mixture, the compositions were determined by atomic absorption technique in some cases and X-ray fluorescence technique in others. When single-phase products were directly obtained, the composition was assumed to be equal to the reactant composition. The unit cell data and the analytical data obtained by atomic absorption were employed using Vegard's rule (L. Vegard, Z. Phys. 5, 17 (1921); Z. Krist. 67, 239 (1928) —see also "Concise Chemical and Technical Dictionary," H. Bennett, Chemical Publishing Co., 1962, i.e.,

35 "when two similar crystalline materials form a solid solution, the lattice constant of this solution divides the space between their respective lattice constants in ratio to their relative quantities") to obtain a unit cell dimension for hypothetical  $\text{CrS}_2$  where  $a=5.593 \pm 0.008$  Å. This value was used to obtain the approximate composition of other phases by using Vegard's rule.

40 The Cr content is a function of the starting ratio of elements and the pressure. When 30 kb. was used, a maximum value of  $x \approx 0.1$  was obtained; however, at 65 kb. a maximum value of  $x \approx 0.4$  was achieved. When atmospheric pressure was used, the value of  $x$  was about 0.01.

45 Magnetic measurements were made using a vibrating sample magnetometer. Measurements were made of magnetization,  $\sigma$ , vs. field,  $H$ , and vs. temperature,  $T^\circ\text{K}$ . The Curie temperature,  $T_c$ , saturation magnetization  $\sigma_s$  in emu./g. were obtained from the data. As  $x$  was increased, the value of  $T_c$  increased while  $\sigma_s$  decreased.

50 These phases exhibit utility in many of the usual applications of magnetic materials such as magnetic switching devices, information storage, transformer coils, etc. They are also useful in applications requiring a range of temperature sensitivity or magnetization since these materials can be made to have such a range when the Cr content is varied.

55 Electrical measurements were made by a four-probe technique on crystalline samples.

## 3

The materials are electrical conductors with resistivities,  $\rho$ , in the range  $10^{-4}$  to  $10^{-3}$  ohm-cm. at room temperature. The variation of resistivity with temperature is very small. One sample was measured from 4.2 K. to 600° K. and the resistivity varied from  $4 \times 10^{-4}$  ohm-cm. to  $5 \times 10^{-4}$  ohm-cm. This feature of small change in resistivity with a large change in temperature is desired and useful in some resistor applications.

## SPECIFIC EMBODIMENTS OF THE INVENTION

The following are non-limitative examples of the invention. Unless otherwise stated, all parts and ratios are atomic weight ratios for cobalt metal and elemental sulfur and molecular weight ratios for chromium compounds.

## EXAMPLE 1



A pellet weighing 0.3872 g. was pressed from a mixture of Co metal powder,  $\text{Cr}_2\text{S}_3$  and elemental sulfur mixed in the ratio 2:1:6. It was pressured to 65 kb. and reacted at 1100° C. for one hour, cooled over a four hour period to 900° and quenched. The product was composed of black, shiny material part of which was magnetic. The magnetic part was separated by passing the powdered sample through a magnet. X-ray diffraction of this sample showed a pattern similar to that of pyrite-type  $\text{CoS}_2$ , but the lines were shifted to lower angles indicating a larger cell. Diffraction lines of excess  $\text{Cr}_2\text{S}_3$  were also in the pattern. The cell was measured and  $a$  was found to equal 5.5495 Å. This value is larger than the cell dimension of  $\text{CoS}_2$  in which  $a=5.5346$  Å.

Using Vegard's rule, the composition of the pyrite-type phase was calculated to be  $\text{Co}_{0.75}\text{Cr}_{0.25}\text{S}_2$ .

## EXAMPLE 2



A pellet weighing 0.3782 g. was pressed from a mixture of 2 parts Co metal powder, one part  $\text{Cr}_2\text{S}_3$  and six parts sulfur. It was pressured to 65 kb. and reacted at 1300° C. for one hour and cooled over a period of two hours to 1200°, and quenched. Four regions of black crystalline material were seen in the pellet. At the very end of the pellet, material which was magnetic at room temperature was present. The X-ray powder patterns showed the presence of  $\text{Cr}_2\text{S}_3$  and a pyrite-type phase of cell dimension  $a=5.544$  Å. Next toward the center, crystals of  $\text{Cr}_2\text{S}_3$  were present. In the center of the pellet another magnetic region was present. The powder pattern showed primarily a pyrite-type phase ( $a=5.558$  Å.) and a trace of  $\text{Cr}_2\text{S}_3$ . The composition of this phase determined using Vegard's rule is  $\text{Co}_{0.6}\text{Cr}_{0.4}\text{S}_2$ . Magnetic measurements showed  $T_c=275$ ° K. and  $\sigma_s=18.6$  emu./g.

Around the center of the pellet another region was present which was composed of  $\text{Cr}_2\text{S}_3$  and a poorly crystalline pyrite-type phase.

## EXAMPLE 3



A mixture of 1 part Co metal powder, one part Cr metal powder, and five parts sulfur, was pelleted, pressured to 30 kb. and reacted at 1200° C. for one hour, cooled over a period of three hours to 900°, and quenched.

## 4

The product contained black regions at the ends of the pellet and plastic sulfur in the center. The black region consisted of large and small crystalline regions. The larger crystals were a pyrite-type phase where  $a=5.540$  Å. The smaller crystals were  $\text{Cr}_2\text{S}_3$ . The composition of the pyrite-type phase derived by Vegard's rule is  $\text{Co}_{0.91}\text{Cr}_{0.09}\text{S}_2$ .

## EXAMPLE 4



10 A mixture of 0.15 part  $\text{CrS}$ , 0.85 part Co and two parts sulfur, was pelleted, pressured to 65 kb., and reacted at 1100° C. for two hours and quenched. The product was a homogeneous single phase material. The X-ray powder diffraction pattern showed only a pyrite-type phase of cell dimension in which  $a=5.5422$  Å. Analysis of the Cr and Co content was done by atomic absorption and indicates the formula to be  $\text{Co}_{0.866}\text{Cr}_{0.134}\text{S}_2$ . By Vegard's rule, the formula is  $\text{Co}_{0.87}\text{Cr}_{0.13}\text{S}_2$ .

Magnetic measurements were made:  $\sigma_s=24.7$  emu./g. and  $T_c=286$ ° K.

## EXAMPLE 5



25 A pellet was pressed from a mixture of 0.35 part  $\text{CrS}$ , 0.65 part Co, and 2.5 parts S, pressured to 65 kb., and reacted at 1300° C. for two hours and quenched. The product consisted of end and center regions. The end regions were composed of black crystals, part of which were magnetic at room temperature and part were magnetic below room temperature. The former part showed primarily a pyrite-type powder pattern but some  $\text{Cr}_2\text{S}_3$  was also present. The latter part showed a pure pyrite-type pattern where  $a=5.5393$  Å. The composition calculated by Vegard's rule is  $\text{Co}_{0.908}\text{Cr}_{0.092}\text{S}_2$ .

30 35 The center region of the pellet contained pyrite-type phase and  $\text{Cr}_2\text{S}_3$ .

## EXAMPLE 6



40 45 A pellet weighing 0.431 g. made from a mixture of 0.636 g. Co, 0.063 g. Cr, and 0.862 g. S was pressured to 65 kb. and heated to 1300° C., held for one hour at 1300° C., cooled at a rate of 50° per hour for four hours to 1100° C. and quenched. The bulk of the product consisted of microcrystalline material. At a region close to the ends of the pellet, larger crystals were separated mechanically. The powder diffraction pattern of these indicated a single phase material of pyrite-type structure with  $a=5.5376$  Å. According to Vegard's rule, the composition is  $\text{Co}_{0.95}\text{Cr}_{0.05}\text{S}_2$ . Magnetic measurements made on these crystals show  $T_c=177$ ° K. and  $\sigma_s=36.53$  emu./g.

## EXAMPLES 7-12

A series of reactions was run starting with various ratios of  $\text{CrS}$ , Co and S. These were pressed into pellets, pressured to 65 kb., and reacted at 1200° C. for two hours and quenched. The products of all reactions consisted of black, rod-like crystals of the pyrite-type phase at the ends of the pellet. In the center, the excess S or  $\text{Cr}_2\text{S}_3$  were present. The crystals were easily separable for chemical analysis, magnetic and electrical measurements. The data are shown in Table I.

TABLE I

| Example | Starting ratio    | Cell dimension in Å. | Composition                                  | Method of determination <sup>1</sup> | Magnetic data        |              | Resistivity          |
|---------|-------------------|----------------------|----------------------------------------------|--------------------------------------|----------------------|--------------|----------------------|
|         |                   |                      |                                              |                                      | $\sigma_s$ , emu./g. | $T_c$ , ° K. |                      |
| 7       | 0.5CrS/0.5CO/2S   | 2.5.5508 (2)         | $\text{Co}_{0.75}\text{Cr}_{0.25}\text{S}_2$ | (a)                                  | 16.2                 | 342          | $3.0 \times 10^{-4}$ |
| 8       | 0.4CrS/0.6CO/2S   | 5.5452 (2)           | $\text{Co}_{0.82}\text{Cr}_{0.17}\text{S}_2$ | (b)                                  | 20.75                | 302          | —                    |
| 9       | 0.35CrS/0.65CO/2S | 5.5494 (1)           | $\text{Co}_{0.75}\text{Cr}_{0.25}\text{S}_2$ | (a)                                  | 16.32                | 343          | —                    |
|         |                   | 5.5456 (1)           | $\text{Co}_{0.81}\text{Cr}_{0.19}\text{S}_2$ | (a)                                  | 20.75                | 302          | —                    |
| 10      | 0.25CrS/0.75CO/2S | 5.5477 (1)           | $\text{Co}_{0.79}\text{Cr}_{0.21}\text{S}_2$ | (a)                                  | 16.77                | 335          | —                    |
|         |                   | 5.5508 (1)           | $\text{Co}_{0.75}\text{Cr}_{0.27}\text{S}_2$ | (a)                                  | —                    | —            | $9.8 \times 10^{-4}$ |
| 11      | 0.20CrS/0.80CO/2S | 5.5450 (1)           | $\text{Co}_{0.83}\text{Cr}_{0.16}\text{S}_2$ | (c)                                  | —                    | —            | $1.1 \times 10^{-3}$ |
| 12      | 0.15CrS/0.85CO/2S | 5.5451 (1)           | $\text{Co}_{0.82}\text{Cr}_{0.18}\text{S}_2$ | (c)                                  | —                    | —            | —                    |

<sup>1</sup> (a) =Vegard's rule; (b) =X-ray fluorescence; (c) =Atomic absorption.

<sup>2</sup> Numbers in parentheses are standard deviations.

## 5

## EXAMPLE 13



A mixture of 0.05 Cr (0.0468 g.) and 0.95 Co (1.0078 g.) was dissolved dilute  $\text{H}_2\text{SO}_4$  (1.5 ml.  $\text{H}_2\text{SO}_4+20$  ml.  $\text{H}_2\text{O}$ ) and nitrogen bubbled through the solution which was heated to speed reaction. The solution was poured into acetone to precipitate the metal sulfates in finely divided and intimately mixed form. The latter mixture was heated to 100° C. in vacuum to remove water of crystallization, then heated at 350° C. in a flowing  $\text{H}_2\text{S}/\text{N}_2$  mixture to produce an intimate mixture of fine particle sulfides. This mixture was sealed in vacuo in a silica tube with a large excess of sulfur and heated at 650° C. for three days and quenched in cold water. Spectroscopic analysis of the product showed 2-10% Cr to be present. X-ray powder diffraction showed a good pyrite pattern with trace amounts of  $\text{Cr}_2\text{S}_3$ . The cell dimension is 5.5353 A. which corresponds approximately to the composition  $\text{Co}_{0.99}\text{Cr}_{0.01}\text{S}_2$  as derived using Vegard's rule. Magnetic measurements showed  $T_c=140$ ° K.

## EXAMPLE 14



A mixture of 0.33 part Cr and 0.667 part Co was prepared in the manner described in Example 13. Excess sulfur was added to produce stoichiometric  $\text{Co}_{0.99}\text{Cr}_{0.01}\text{S}_2$ . The mixture was sealed in a gold tube and heated for six hours at 3000 atm. pressure and 700° C. and then cooled. The product was extracted with carbon disulfide to remove unreacted sulfur and gave a black powder. The product was magnetic when cooled to liquid nitrogen temperature. The Debye-Scherrer pattern showed the presence of a pyrite phase ( $a=5.5350$  A.),  $\text{Cr}_2\text{S}_3$ , and unidentified material. The cell dimensions of the phase indicate some Cr substitution, and had an approximate composition using Vegard's rule of  $\text{Co}_{0.99}\text{Cr}_{0.01}\text{S}_2$ .

## 6

## EXAMPLE A

The product of Example 5 which was magnetic below room temperature was used in a thermomagnetic switching device. The end region of the pellet which showed a pure pyrite-type pattern of cell constant  $a=5.5393$  A. which corresponds to composition  $\text{Co}_{0.998}\text{Cr}_{0.092}\text{S}_2$  was used. It was mounted using silver paste to a brass spring positioned opposite to a conducting contact and the assembly placed between the poles of a horseshoe magnet. An ohm meter was placed in series with the spring and the conducting contact.

When the device was cooled below room temperature the product became magnetic and the force of the magnetic material overcame the force of the spring, thus causing contact. Current flowed through the circuit as indicated by the ohm meter. The compounds of the invention are therefore useful as temperature sensing agents and may be used to construct switching devices for various purposes, i.e. thermostats, fire alarms, and the like.

What is claimed is:

1. A magnetic composition of the formula  $\text{Co}_{1-x}\text{Cr}_x\text{S}_2$  where  $x=0.01$  to 0.4 having the pyrite-type structure.
2. The composition of claim 1 wherein  $x=0.25$ .
3. The composition of claim 1 wherein  $x=0.4$ .
4. The composition of claim 1 wherein  $x=$ about 0.09.
5. The composition of claim 1 wherein  $x=.13$ .
6. An electrical switching device containing a composition of claim 1 as a temperature sensing agent.

## References Cited

## UNITED STATES PATENTS

3,372,997 3/1968 Bither ----- 23—315

TOBIAS E. LEVOW, Primary Examiner

J. COOPER, Assistant Examiner

U.S. CL. X.R.

23—134; 335—146